

# UNITED STATES PATENT OFFICE.

GEORG HEBERLEIN, OF WATTWIL, SWITZERLAND.

## PROCESS FOR THE PRODUCTION OF PATTERN EFFECTS UPON COTTON FABRICS.

1,201,961.

Specification of Letters Patent.

Patented Oct. 17, 1916.

No Drawing.

Application filed February 17, 1916. Serial No. 79,005.

*To all whom it may concern:*

Be it known that I, GEORG HEBERLEIN, chemist, a citizen of the Swiss Republic, and resident of Wattwil, Canton of St. Gall, Switzerland, have invented a new and useful Process for the Production of Pattern Effects upon Cotton Fabrics, of which the following is a full, clear, and exact specification.

10 The invention relates to modifications of the process for the production of pattern effects upon cotton fabrics described in my United States Letters Patent No. 1144655 dated 29th June 1915.

15 I have found that the transparent effects produced upon mercerized cotton fabrics by the short local action of sulfuric acid of over 50 $\frac{1}{2}$ ° Baumé is enhanced if the fabric be submitted to subsequent mercerization by 55 soda lye.

20 The process as improved consists therefore firstly in submitting the fabric to mercerization by means of soda lye; secondly in printing the fabric thereafter with sulfuric acid of over 50 $\frac{1}{2}$ ° Baumé and washing out after a few seconds, or, printing upon the fabric in a resist and passing it through concentrated sulfuric acid of over 50 $\frac{1}{2}$ ° Baumé for a few seconds, and thereafter 65 washing it out, and finally in submitting the fabric to a further mercerization with soda lye.

25 Transparent effects similar to those described in the United States Letters Patent 70 No. 1144655 may also be secured by printing the fabric with sulfuric acid of over 50 $\frac{1}{2}$ ° Baumé and washing it out after a few seconds or by printing upon the fabric in a resist and then passing it for a few seconds 75 through concentrated sulfuric acid of over 50 $\frac{1}{2}$ ° Bé. and then washing, and subsequently

submitting the fabric to mercerization with soda lye.

What I claim is:

1. The described process for obtaining 45 pattern effects upon cotton fabrics consisting of taking mercerized fabrics, subjecting the parts where pattern effects are to be produced for a few seconds to the action of sulfuric acid of over 50 $\frac{1}{2}$ ° Bé., washing out 50 the acid and finally subjecting the fabrics to a further mercerization with soda lye.

2. The described process for obtaining pattern effects upon cotton fabrics consisting of taking mercerized fabrics, printing 55 the required pattern on the said mercerized cotton fabrics with sulfuric acid of over 50 $\frac{1}{2}$ ° Bé., washing out the acid after a few seconds and finally subjecting the fabrics to a further mercerization with soda lye. 60

3. The described process for obtaining pattern effects upon cotton fabrics consisting of subjecting the parts of the fabrics where pattern effects are to be produced for a few seconds to the action of sulfuric acid 65 of over 50 $\frac{1}{2}$ ° Bé., washing out the acid and finally subjecting the fabrics to a mercerization with soda lye.

4. The described process for obtaining pattern effects upon cotton fabrics consisting of printing the required pattern on the fabrics with sulfuric acid of over 50 $\frac{1}{2}$ ° Bé., washing out the acid after a few seconds and finally subjecting the fabrics to a mercerization with soda lye. 75

In witness whereof I have hereunto signed my name this 4th day of January, 1916, in the presence of two subscribing witnesses.

DR. GEORG HEBERLEIN.

Witnesses:

A. BAUMRATZ,  
E. GATTB.